

## UNITED STATES PATENT OFFICE

2,010,423

METHOD OF MANUFACTURING ASPHALT  
AND PRODUCT THEREOFAlfred A. Wells, Roselle Park, N. J., assignor to  
Standard Oil Development Company, a corpo-  
ration of DelawareNo Drawing. Application September 1, 1932,  
Serial No. 631,369

6 Claims. (Cl. 196—74)

This invention relates to a new and improved method in the art of manufacturing asphalt by blending heavy petroleum hydrocarbons. More particularly, this invention relates to emulsifying fluxes, which are prepared according to this invention by blending high melting point asphalt with an extract derived from a cylinder oil fraction from the same crude from which the asphalt was derived or from another crude; the said extract being obtained by extracting with either phenol, sulfur dioxide, furfural or similar solvents.

In refining oils it is often-times necessary or desirable to produce both cylinder stock and asphaltic material from the same crude. This is the case in the distillation of Colombian, coastal and mid-continent crudes as well as others, where, in order to obtain maximum yields of cylinder stock, it is necessary to reduce the asphalt to a high melting point. For many purposes, for example, in the manufacture of asphalt emulsions, etc., it is necessary that the asphaltic material have a comparatively low melting point. In some instances, for example, Colombian crude, the lubricating oil fraction contains comparatively large quantities of organic acidity.

An object of this invention is to produce a maximum yield of a cylinder stock and of an asphalt of low melting point from the same crude.

Another object of this invention is the production of a cylinder oil of low organic acidity.

These and other objects of the invention will be understood by the following description:

A crude oil such as Colombian crude for example, after the removal of the lighter oil fraction, is subjected to further heat to distill the maximum amount of cylinder oil. The cylinder oil fraction is then extracted with sulfur dioxide, phenol or furfural or similar selective solvents to give higher A. P. I. gravity, improved viscosity index and better stability, that is more resistant to oxidation, than other methods of treatment. The extracted material is separated from the solvent and incorporated with the asphaltic residue. It is desirable in some cases to redistill the extracted oil so as to give a higher viscosity blending stock; caustic such as sodium hydroxide may be incorporated during distillation if desired to remove any organic acids or solvent that may still be present in the oil. The characteristics of finished asphalt will vary with proportions of extract and high melting asphalt. The mixture of asphalt and solvent extract may then be used as such or it may be used in making emulsions upon the addition of caustic soda and oleic acid. Other

emulsifying agents other than caustic soda and oleic acid may be substituted.

By this method, it has been found that the extracted material can be blended with high melting point asphalt in proper proportion so as to give a final product which is equivalent to or superior to the asphaltic product which would have been obtained on straight reduction to the desired melting point. This product is superior over other asphalts in that it is a better emulsifying asphalt with a better softening point penetration relationship and also a better softening point ductility relationship.

The penetration characteristics vary with the melting point of the flux, i. e., the oil content. This method allows the manufacturer exact control so that he can vary his product to meet special requirements, which up to the present have required processing special crude oils to meet special requirements. It is, of course, evident that material extracted from cylinder oil from one crude can be blended with asphalt from other sources of a mixture. The reverse is also true. If desired, the asphalt may also be oxidized.

Another advantage of this method is improving the maximum yield of cylinder stock from different crudes.

Various changes may be made within the scope of the appended claims in which it is desired to claim all novelty inherent to the invention as broadly as the prior art permits.

I claim:

1. An asphalt comprising a mixture of asphaltic residues obtained from the distillation of petroleum oil containing an extract obtained from a solvent extraction of the higher boiling fractions of the same petroleum oil with an organic solvent that is liquid at atmospheric pressure and temperature, of the group consisting of phenol and furfural.

2. A method of manufacturing asphalts which comprises subjecting a crude oil to distillation, separating the lighter and the higher boiling fractions from an asphaltic residue, subjecting the higher boiling fractions to solvent extraction with an organic solvent that is liquid at atmospheric pressure and temperature, of the group consisting of phenol and furfural, separating the extracted material from the solvent and mixing the extracted material with the said asphaltic residue.

3. A method of manufacturing asphalts which comprises subjecting a crude petroleum oil to distillation to separate the lower and higher boil-

ing fractions from the asphaltic material present in the crude, extracting by the use of organic solvents that are liquid at atmospheric pressure and temperature of the group consisting of phenol and furfural the soluble portion of the highest boiling point overhead portion obtained by the distillation of the crude petroleum oil, separating the solvent from the extracted material and mixing the said asphaltic residue and the said extracted material.

4. Method of manufacturing asphalts according to claim 3 in which the solvent used in extracting the high boiling point oil is phenol.

5. Method of manufacturing asphalts accord-

ing to claim 3 in which the solvent used in extracting the high boiling point oil is furfural.

6. Method of manufacturing asphalts which comprises subjecting a crude petroleum oil to distillation and separately removing as a distillate the volatile fractions including a cylinder oil fraction, subjecting the cylinder oil fraction to solvent extraction using an organic solvent that is liquid at atmospheric pressure and temperature, of the group consisting of phenol and furfural, separating the solvent and the extracted material, and incorporating the asphaltic residue with the extracted material.

ALFRED A. WELLS.